

L. W. COLBURN.

METHOD AND APPARATUS FOR DRAWING WIRE GLASS,  
APPLICATION FILED FEB. 28, 1917, RENEWED JUNE 11, 1919.

1,323,339.

Patented Dec. 2, 1919.



Inventor  
Irving W. Colburn  
By Whittemore, Hubbell & Whittemore  
Atty's

I. W. COLBURN.

METHOD AND APPARATUS FOR DRAWING WIRE GLASS.

APPLICATION FILED FEB. 28, 1917. RENEWED JUNE 11, 1919.

1,323,389.

Patented Dec. 2, 1919.

2 SHEETS—SHEET 2.



Inventor  
Irving W Colburn  
By Whittamor Hubert & Whittamore

Atty

# UNITED STATES PATENT OFFICE.

IRVING W. COLBURN, OF TOLEDO, OHIO, ASSIGNOR TO THE LIBBEY-OWENS SHEET GLASS COMPANY, OF TOLEDO, OHIO, A CORPORATION OF OHIO.

## METHOD AND APPARATUS FOR DRAWING WIRE-GLASS.

1,323,389.

Specification of Letters Patent.

Patented Dec. 2, 1919.

Application filed February 28, 1917, Serial No. 151,582. Renewed June 11, 1919. Serial No. 303,474.

To all whom it may concern:

Be it known that I, IRVING W. COLBURN, a citizen of the United States of America, residing in the city of Toledo and county of Lucas, State of Ohio, have invented certain new and useful Improvements in Methods and Apparatus for Drawing Wire-Glass, of which the following is a specification, reference being had therein to the accompanying drawings.

This invention relates to the art of making sheet glass. The object of the invention is to provide a process and apparatus whereby sheet glass of uniform width and thickness may be drawn from the molten mass and a wire mesh or wire cloth may be drawn in the sheet so as to make what is known as "wire glass;" all as more fully herein-after described and specifically pointed out in the claims.

In the drawings Figure 1 is a vertical central longitudinal section through a machine embodying my invention and Fig. 2 is a partial side elevation of the same.

The invention in general as shown herein may be substantially of the type shown in my pending application Serial Number 54,714, filed October 8, 1915, in which the glass is drawn horizontally from the tank, and comprises a drawing table, A, which may be of the type shown in that application or in my Patent No. 1,122,192, issued December 29, 1914, which, as well known, comprises endless chains, one supported in a horizontal plane and the other pressing upon it from above and drawing it from the tank and delivering it to the leer. I also provide a melting tank, B, and a cooling chamber, C, in which the glass may be more or less tempered, and a drawing chamber, D, the back of which may be formed by a tile, E, forming a narrow trough-like body of glass from the front edge of which the sheet, F, is drawn by the drawing table. I

show below the tile E a heating chamber, G, and a valve, H, which may be raised more or less above the surface of the glass to assist in controlling the temperature at the drawing point. A pair of rolls, I, are situated a short distance from the edge of the drawing table, these rolls being driven and being hollow for the purpose of cooling. The surface may be plain or figured, as desired.

I also show a driven supporting roller,

K, and another driven supporting roller, L, between the rolls I and the drawing table A. I also show cooling chambers, M, through which water may be circulated above and below the sheet between the rolls I and K.

O is a gas pipe for supplying flame, if desired, to the drawing edge.

P is the heating chamber for discharging the heat into the drawing chamber.

Q is a roof which may extend over the span between the drawing chamber and the tank.

R is a roller, preferably of vitrified material and preferably driven, although it may be an idler, the lower edge of which dips into the glass, as plainly shown in the drawings. Above this roller is a slot, S, through which passes a wire cloth, T, being held from contact with the walls by a roller, T'. The wire cloth as shown is supported on a roller, U, above the tank, and the same being led down through the slot S and over the roller R and carried beneath the surface of the glass between the rolls I, will be drawn into the sheet midway between the surfaces as the sheet is drawn, as clearly indicated in the drawings.

Having thus described my invention, what I claim as new and desire to secure by Letters Patent is:

1. The method of drawing wire glass consisting in guiding the wire cloth into the mass of molten glass, drawing the molten glass in sheet form, horizontally, parallel with the surface, with the wire cloth embedded therein.

2. In an apparatus for drawing wire glass the combination of a guide for leading wire cloth into the mass below the surface and means for drawing the sheet of glass along the plane of the surface of the mass with the embodied wire mesh.

3. In an apparatus for drawing wire glass the combination of a drawing chamber having a slot in the roof thereof through which a wire cloth is adapted to be drawn, a roll in the drawing chamber under which the wire cloth passes, the lower point of the roll dipping into the glass, and drawing means for drawing the sheet glass and embedded wire horizontally in line with the bottom of the roll.

4. In a wire glass drawing apparatus, the combination of a drawing chamber having

an open end, a pair of drawing rolls adjacent thereto adapted to receive and draw a glass sheet horizontally from the top of the glass at the open end of the drawing chamber, and a guide for a wire cloth beneath the surface of the glass in the drawing chamber to a point in line with the space between the rolls.

5. In an apparatus for forming wire glass, 10 the combination of a tank having an overflow outlet passage arranged for the flow of glass in a sheet, and means for directing a wire fabric into the glass in the tank and feeding it along said passage with the flow 15 of glass.

6. In an apparatus for forming wire glass, 20 the combination of a tank having an overflow outlet passage arranged for the flow of glass in a sheet, means for directing a wire fabric into the glass in the tank and feeding it along said passage with the flow of 25 glass, and means beyond the outlet to support and draw the sheet of glass in the direction in which it moves through the passage.

7. In an apparatus for forming wire glass, 30 the combination of a melting tank having an outlet arranged for a flow of glass from the surface of the pool in a continuous sheet, means to direct a wire fabric into the glass in the tank and with the flowing glass 35 through said outlet.

8. In sheet glass forming apparatus, the 35 combination of a tank for molten glass having a horizontal overflow surface just below the normal surface of the glass, arranged to permit the glass to move in a continuous sheet thereover, means to direct a wire fabric into the glass in the tank and along said 40 overflow surface beneath the surface of the glass, and means beyond the outlet to support and draw the sheet.

9. In sheet glass forming apparatus, the 45 combination of a tank for molten glass, means to feed a wire fabric downward into

the molten glass in the tank, and means to draw a sheet of glass with the wire fabric embedded therein horizontally from the tank.

10. In sheet glass forming apparatus, the 50 combination of a tank for molten glass, sheet drawing means beyond the tank for drawing the glass horizontally from the tank in a continuous sheet at the level of the glass in the tank, and means to direct 55 a wire fabric into the tank horizontally just below the surface of the glass to the sheet drawing means, whereby the fabric is embedded in the sheet and drawn therewith.

11. In sheet glass forming apparatus, the 60 combination of a tank for molten glass, having a horizontal overflow outlet extension at the level of the glass, permitting the glass to flow in a continuous sheet thereover, sheet drawing means beyond the tank for drawing the glass in a sheet from said outlet, means for embedding a wire fabric in the sheet, comprising a roll dipping into the glass in the tank, and around the under surface of which the fabric is guided and from 65 which it extends to the sheet feeding means.

12. The method of forming wire glass, 70 which consists in flowing molten glass in a continuous sheet from the surface of a pool of glass, drawing the glass as it passes beyond the tank, directing a wire fabric into the tank, and causing it to advance with the flow of glass.

13. The method of forming wire glass, 75 which consists in drawing a sheet of glass 80 horizontally from the surface of a pool of molten glass and directing a wire fabric into the pool, and thence horizontally with the flow of glass from the pool.

In testimony whereof I affix my signature 85 in presence of two witnesses.

IRVING W. COLBURN.

Witnesses:

IDA E. COLBURN,  
JAMES HOVEY.